

1

3,625,697

## SENSITIZATION OF LIGHT-SENSITIVE SILVER HALIDE PHOTOGRAPHIC EMULSIONS

Shui Sato and Rintaro Ushiyama, Tokyo, Eiichi Sakamoto, Hanno-shi, and Sadatugu Terada and Hiroshi Yamada, Tokyo, Japan, assignors to Konishiroku Photo Industry Co., Ltd., Tokyo, Japan

No Drawing. Filed Dec. 10, 1969, Ser. No. 884,022  
Claims priority, application Japan, Dec. 13, 1968,

43/90,990

Int. Cl. G03c 1/28, 1/34

U.S. Cl. 96—107

5 Claims

### ABSTRACT OF THE DISCLOSURE

Light-sensitive silver halide emulsions are sensitized by incorporating into the emulsion, a sensitizing amount (0.1–1000 mg./kg.) of a compound of the formula:



wherein A is a lower alkylene group, or a polyalkylene ether group, having the formula:

$—(\text{CH}_2\text{CH}_2\text{O})_p—$ ,  $—(\text{CH}_2\text{CH}_2\text{O})_p—\text{CH}_2—\text{CH}_2$  or  $—(\text{CHCH}_2\text{O})_p—$   
and which is not bonded through an oxygen atom to B; A' is a lower alkylene group, or a polyalkylene ether group having the formula



provided that A and A' are not both polyalkylene ether groups at the same time, and p is an integer of 2 to 30; B and B' are  $—\text{NH}$ — or  $—\text{O}$ —, provided that both are not  $—\text{O}$ — at the same time; R is a lower alkyl group, a phenyl group, an aralkyl group or  $—(\text{CH}_2)_q—\text{COOR}'$ , wherein q is an integer of 1 to 3, and R' is a lower alkyl group; and X is a divalent group of the formula:



is a lower alkyl group.

This invention relates to a light-sensitive silver halide photographic emulsion sensitized by incorporating therein a sulfur-containing compound which will be described below.

Numerous methods are known for the sensitization of light-sensitive silver halide photographic emulsions. Typical of these is chemical sensitization using either a sulfur compound capable of yielding a silver sulfide or a suitable reducing compound; or a noble metal salt. Further, it is well known that the joint use of said compounds can further increase the sensitivity of the emulsion (refer, for example, to The Theory of the Photographic Process, third edition (1967), pages 113–117).

However, the known chemical sensitization process of this kind is severely restricted as far as the amount of the compound to be added, and has such disadvantages that if the amount exceeds a definite limit, the emulsion is greatly increased in fog and becomes low in stability during storage of the resulting film at an elevated temperature. Further, if a photographic emulsion is subjected to high temperature ripening in the presence of such a sensitizer as mentioned above, usually, only fogging of the emulsion is increased while the desired increase in sensitivity can not be attained after a definite sensitivity has been reached.

2

The object of the present invention is to provide silver halide photographic emulsions improved in photographic properties, which are less in fog formation and which are increased in sensitivity.

As the result of various studies, we have found that the above object can be effectively achieved by applying the novel sensitizing compounds mentioned below to silver halide photographic emulsions.

The compounds employed in the present invention have many characteristics different from those of the conventional chemical sensitizers. For example, they are usable as additives prior to coating and, when used in combination with chemical sensitizers, they can further increase the sensitivity of silver halide photographic emulsions without any accompanying fog formation.

The sensitizing compounds useful in the present invention are represented by the formula



wherein A is a lower alkylene group, or a polyalkylene ether group of the formula  $—(\text{CH}_2\text{CH}_2\text{O})_p—$ ,



and which is not bonded through an oxygen atom to B; A' is a lower alkylene group, or a polyalkylene ether group of the formula  $—(\text{CH}_2\text{CH}_2\text{O})_p—\text{CH}_2—\text{CH}_2—$  or



provided that A and A' are not both polyalkylene ether groups at the same time, and p is an integer of 2 to 30;

35 B and B' are  $—\text{NH}$ — or  $—\text{O}$ —, provided that both are not  $—\text{O}$ — at the same time;

R is a lower alkyl group, a phenyl group, an aralkyl group or  $—(\text{CH}_2)_q—\text{COOR}'$ , wherein q is an integer of 1 to 3 and R' is a lower alkyl group; and

40 X is a divalent group of the formula  $—\text{S}—, —\text{O}—,$



45 wherein R'' is a lower alkyl group.

Typical examples of the above-mentioned compounds are as follows:



## 3



Synthesis examples of several compounds among three mentioned above are set forth immediately below.

## SYNTHESIS EXAMPLE 1

## Synthesis of the compound (1):

A solution of 17.8 g. of  $\text{HOCH}_2\text{CH}_2\text{SCH}_2\text{CH}_2\text{COOC}_2\text{H}_5$  in 100 cc. of dry benzene was added with 8.6 g. of  $\text{S}(\text{CH}_2\text{CH}_2\text{NCO})_2$ . The mixture was refluxed for 2 hours and was then freed from the solvent by distillation under reduced pressure. The residue was dissolved in 200 cc. of ether, and was cooled and recrystallized to obtain the compound (1), M.P. 45°–46° C.

## SYNTHESIS EXAMPLE 2

## Synthesis of the compound (5):

A solution of 7.3 g. of  $\text{CH}_3\text{—N}(\text{CH}_2\text{CH}_2\text{CH}_2\text{NH}_2)_2$  in dry benzene was added with 13.1 g. of



The mixture was refluxed for 2 hours in a water bath and was then cooled to deposit a crystalline mass. This mass was recrystallized from benzene to obtain the compound (5), M.P. 82°–83° C.

## SYNTHESIS EXAMPLE 3

## Synthesis of the compound (6):

A solution of 15 g. of  $\text{HO}(\text{CH}_2\text{CH}_2\text{O})_{13}\text{H}$  in 50 cc. of dry benzene was added with 6.1 g. of



The mixture was refluxed for 8 hours and then the benzene was removed by distillation under reduced pressure

70

## 4

to obtain the compound (6) in the form of a slightly yellow transparent solution,  $n_D^{23}$  1.4873.

## SYNTHESIS EXAMPLE 4

5 Synthesis of the compound (12):  
A solution of 13.6 g. of

10

in dry benzene was gradually added with 26.2 g. of  $\text{C}_2\text{H}_5\text{SCH}_2\text{CH}_2\text{NCO}$ . The mixture was refluxed for 3 hours and was then cooled to deposit a crystalline mass. This mass was recovered by filtration and was recrystallized from methanol to obtain the compound (12), M.P. 207°–208° C.

Other compounds than those mentioned above can also be synthesized according to the above-mentioned synthesis examples.

20 The thus obtained compounds employed in the present invention may be added to emulsions at any stage during the second ripening. Most desirably, however, they are preferably added at the beginning of the second ripening. Silver halide emulsions containing these compounds are 25 increased in gamma, photographic speed and maximum density and make is possible to obtain light-sensitive photographic materials having improved storability.

The above-mentioned compound useful in the present invention may be added to a silver halide emulsion after 30 dissolving the compound in water or in a water-miscible organic solvent such as methanol or ethanol. The amount of the compound to be added varies depending on the kind of the compound or of the silver halide emulsion employed, but is ordinarily in the range of 0.1 mg.–1000 35 mg. per kg. of silver halide emulsion.

The compounds employed in the present invention are applicable to all types of silver halide emulsions such as silver chlorobromide emulsion, silver iodobromide emulsion, etc. Further the emulsions may have been subjected 40 to gold sensitization or sulfur sensitization, and may have been incorporated with spectral sensitizers, polyalkylene oxide type sensitizers, various stabilizers, hardeners and coating aids.

The compounds employed in the present invention can 45 be applied not only to monochromatic photographic emulsions but also to color photographic emulsions containing oil-soluble or water-soluble color couplers.

The silver halide photographic emulsions of the present 50 invention which are obtained in the above-mentioned manner are coated onto common supports such as, for example, glass; cellulose triacetate film bases, polyester film bases or baryta papers.

The present invention is illustrated in further detail 55 below with reference to examples, but the invention is not limited to these examples.

## EXAMPLE 1

A silver halide emulsion comprising 2 mole percent of silver iodide and 98 mole percent of silver bromide was 60 subjected to second ripening by the use of a sulfur sensitizer and a gold sensitizer to prepare a silver iodobromide emulsion for high speed photographic negatives. This emulsion was divided into portions of 100 g. each, and the divided emulsions were individually incorporated with the present compounds set forth in Table 1 below. The thus treated emulsions were coated onto cellulose triacetate film bases and were then dried to prepare samples.

For comparison, the compound



disclosed in U.S. Pat. No. 3,021,215 was treated in the same manner as above to prepare a control sample.

These samples were exposed to light by means of a sensitometer KS-1 (manufactured and sold by Konishiroku Photo Industry Co., Ltd.) at 160 Lux-5400° K., and

were then developed at 20° C. for 5 minutes with a developer having the following composition:

|                                |      |
|--------------------------------|------|
| Metol                          | 3    |
| Anhydrous sodium sulfite       | 50   |
| Hydroquinone                   | 6    |
| Sodium carbonate (monohydrate) | 29.5 |
| Potassium bromide              | 1    |
| Water to make 1 liter.         |      |

(The developer was used after dilution with water to 1:1.)

Thereafter, the samples were subjected to sensitometry 20 to obtain the results shown in Table 1.

TABLE I

| Incorporated compound   | Amount (mg./100 g. emulsion) | Speed | Gamma | Maximum density | Fog  |
|-------------------------|------------------------------|-------|-------|-----------------|------|
| Compound (2)            | 50                           | 120   | 0.95  | 2.25            | 0.06 |
| Compound (8)            | 50                           | 130   | 0.95  | 2.27            | 0.07 |
| Compound (10)           | 50                           | 125   | 1.00  | 2.30            | 0.07 |
| Control sample          | 50                           | 120   | 0.88  | 2.05            | 0.09 |
| Non-incorporated sample | 100                          |       | 0.80  | 2.02            | 0.09 |

NOTE.—In the table, the speed is a relative value measured by assuming as 100 the speed of the non-incorporated sample.

As is clear from Table 1, light-sensitive photographic materials improved in speed, gamma and maximum density can be obtained by the use of the silver halide photographic emulsions in accordance with the present invention.

## EXAMPLE 2

A neutral photographic emulsion for photographic negatives, which comprised 5 mole percent of silver iodide and 95 mole percent of silver bromide, was added with given amounts of a sulfur sensitizer and a gold sensitizer, and was then divided into portions of 100 g. each. The divided emulsions were individually incorporated with the present compounds set forth in Table 2 below. Each emulsion was maintained at 56° C. and was subjected to second ripening so as to attain the maximum density. Subsequently, 20 mg. per 100 g. of the emulsion of 4-hydroxy-6-methyl-1,3,3a,7-tetrazaindene were added, and then suitable amounts of a film hardener and a coating aid were added. The thus treated emulsions were uniformly coated onto cellulose triacetate film bases and were then dried to prepare samples. These samples were subjected to storage test, and were then subjected to sensitometry in the same manner as in Example 1 to obtain the results as set forth in Table 2.

then added as a magenta coupler a given amount of a dispersion prepared by dissolving at an elevated temperature 1 - (2,4,6 - trichlorophenyl)-3-[3-(2,4-di-tert-amylphenoxyacetamide) benzamide] - 5 - pyrazolone in a mixture comprising di-n-butyl phthalate and ethyl acetate, and then dispersing the solution in a gelatine solution by means of sodium alkylbenzenesulfonate. This emulsion was thoroughly stirred and was then adjusted to pH 6.8 to obtain a color photographic emulsion.

Emulsions obtained in the above manner were immediately coated uniformly onto cellulose triacetate film bases and were then dried to prepare samples. These samples were exposed in the same manner as in Example 1 and were then developed at 21° C. for 10 minutes with 15 a color developer of the following composition:

|                                                                       |      |
|-----------------------------------------------------------------------|------|
| N-Ethyl-N-β-methanesulfonamidoethyl - 3 - methyl-aminoaniline sulfate | G.   |
|                                                                       | 2.5  |
| Anhydrous sodium sulfite                                              | 2.0  |
| Benzyl alcohol                                                        | 3.8  |
| Sodium hexametaphosphate                                              | 2.0  |
| Sodium carbonate (monohydrate)                                        | 50.0 |
| Potassium bromide                                                     | 1.0  |
| Caustic soda                                                          | 0.6  |
| Water to make 1 liter.                                                |      |

Thereafter, the samples were subjected to ordinary bleaching, fixing and water-washing treatments and then to sensitometry to obtain the results as shown in Table 3.

| Incorporated compound   | Amount (mg./100 g. emulsion) | Speed | Gamma | Fog  |
|-------------------------|------------------------------|-------|-------|------|
| Compound (1)            | 1.5                          | 125   | 0.85  | 0.03 |
| Compound (3)            | 1.5                          | 130   | 0.07  | 0.03 |
| Non-incorporated sample | 100                          |       | 0.65  | 0.03 |

NOTE.—In the table, the speed is a relative value measured by assuming as 100 the white light speed of the non-incorporated sample.

As is clear also from Table 3, the silver halide photographic emulsions according to the present invention give, even when used in combination with a magenta coupler, color photographic materials which are high in sensitivity and less in fog.

What we claim is:

1. A light-sensitive silver halide photographic emulsion comprising, as a sensitizer, a sensitizing amount of a compound having the formula

TABLE 2

| Incorporated compound   | Amount (mg./100 g. emulsion) | Incubated at room temperature for 3 days |                 |      | Incubated at 55° C. for 3 days |                 |      | Incubated at 55° C. relative humidity 80% for 3 days |                 |      |
|-------------------------|------------------------------|------------------------------------------|-----------------|------|--------------------------------|-----------------|------|------------------------------------------------------|-----------------|------|
|                         |                              | Speed                                    | Maximum density | Fog  | Speed                          | Maximum density | Fog  | Speed                                                | Maximum density | Fog  |
| Compound (4)            | 1.0                          | 125                                      | 2.35            | 0.05 | 125                            | 2.32            | 0.07 | 130                                                  | 2.30            | 0.07 |
| Compound (7)            | 1.0                          | 140                                      | 2.40            | 0.07 | 135                            | 2.42            | 0.08 | 135                                                  | 2.41            | 0.06 |
| Compound (11)           | 1.0                          | 115                                      | 2.30            | 0.04 | 120                            | 2.32            | 0.05 | 115                                                  | 2.30            | 0.05 |
| Non-incorporated sample | 100                          |                                          | 2.02            | 0.08 | 105                            | 2.08            | 0.08 | 100                                                  | 2.05            | 0.07 |

(In the table, the speed is a relative value measured by assuming as 100 the speed of the non-incorporated sample.)

From the above table, it is clear that the silver halide photographic emulsions in accordance with the present invention give light-sensitive photographic materials which, even when stored under severe conditions, are less subject to formation of fog and free from any decrease in speed.

## EXAMPLE 3

To a silver iodobromide color photographic emulsion containing 4 mole percent of silver iodide were added given amounts of chemical sensitizers according to sulfur sensitization and gold sensitization, and then the emulsion was divided into portions of 100 g. each. The thus divided emulsions were individually incorporated with the compounds as shown in Table 3.

After being subjected to second ripening so as to attain the optimum properties, each emulsion was charged with the same stabilizer as in Example 2. To this emulsion was

60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
58

provided that A and A' are not both polyalkylene ether groups at the same time, and p is an integer of 2 to 30; B and B' are —NH— or —O—, provided that both are not —O— at the same time;

R is a lower alkyl group, a phenyl group, an aralkyl group or —(CH<sub>2</sub>)<sub>q</sub>—COOR', wherein q is an integer of 1 to 3, and R' is a lower alkyl group; and

X is a divalent group of the formula —S—, —O—,



wherein R'' is a lower alkyl group.

2. A light-sensitive silver halide photographic emulsion as claimed in claim 1, further comprising a color former.

3. A light-sensitive silver halide photographic emulsion as claimed in claim 1, further comprising at least one other known chemical and/or spectral sensitizer.

4. A light-sensitive silver halide photographic emulsion as claimed in claim 1, further comprising at least one

photographic additive selected from the group consisting of stabilizers and hardeners.

5. A light-sensitive silver halide photographic emulsion as claimed in claim 1, wherein the sensitizer is present in an amount of 0.1 to 1000 mg. per kg. of silver halide emulsion.

#### References Cited

#### UNITED STATES PATENTS

|    |           |        |                 |       |        |
|----|-----------|--------|-----------------|-------|--------|
| 10 | 2,739,060 | 3/1956 | Lowe et al.     | ----- | 96—107 |
|    | 3,021,215 | 2/1962 | Williams et al. | ----- | 96—107 |
|    | 3,046,129 | 7/1962 | Graham et al.   | ----- | 96—107 |

NORMAN G. TORCHIN, Primary Examiner

15 R. FICHTER, Assistant Examiner

U.S. CL. X.R.

96—109